

## UNITED STATES PATENT OFFICE.

RAYMOND C. BENNER, OF BAYSIDE, NEW YORK, ASSIGNOR, BY MESNE ASSIGNMENTS, TO THE PREST-O-LITE COMPANY, INC., OF NEW YORK, N. Y., A CORPORATION OF NEW YORK.

## SEPARATOR AND METHOD OF MAKING THE SAME.

No Drawing.

Application filed May 2, 1922. Serial No. 557,906.

To all whom it may concern:

Be it known that I, RAYMOND C. BENNER, a citizen of the United States, residing at Bayside, in the county of Queens and State 5 of New York, have invented certain new and useful Improvements in Separators and Methods of Making the Same, of which the following is a specification.

This invention relates to an improved 10 storage battery separator and methods of making the same.

Thin sheets of wood, now generally employed in the manufacture of storage battery separators, are usually treated to free the 15 wood of detrimental substances and have been impregnated with various materials to make them less subject to deterioration before service, and more durable in service. However, wooden separators have certain 20 distinct advantages, for example their lightness and the low resistance they offer to the current in the battery but, in their natural condition and even after treatment, they vary considerably in degree of porosity, in 25 strength, in impurities which may be injurious in the operation of the battery, frequently warp and split because of the grain therein, and are also rather expensive, especially if they are selected to obtain uniform 30 high quality separators.

The object of this invention is to provide an improved separator that is light and offers a low resistance to current, but is of uniform strength, uniformly porous, rigid, acid-resistant, less expensive than wood, and free from deleterious substances.

Relatively cheap fibrous materials, desirably those which have been chemically treated and are entirely freed from substances 40 which are or may be detrimental in the battery, are used as the raw materials for making the body of the improved separator. Sulfite pulp and cotton linters are examples of such materials. Sulfite pulp, as 45 is well known, is made from wood in large quantities as a raw material for the paper-making industry and is therefore readily obtainable on the market conditioned for use in separators having the deleterious substances such as resins, gums and acetic acid 50 forming agents already removed therefrom. Cotton linters are likewise readily obtainable as raw material, either chemically

treated or not, as desired. The sulfite pulp, as well as the cotton linters, principally consist of relatively long fibers which may be loosely felted into sheets of the desired thickness and porosity by well known methods, and accordingly a separator that is uniform as to its strength, porosity and freedom from detrimental constituents may readily be obtained by properly controlling the fabrication of such sheets.

In order that the sheet or body of fibrous material shall have the requisite rigidity for service, as in a storage battery separator, suitable bonding and reinforcing material is incorporated either in the chemically treated fibrous material before it is formed into the sheet or into the sheet after it has been 70 formed of such fibrous material.

For example, non-conductive acid-resistant plastic bonding agents such as rubber, celluloid and asphalt may be mixed with fibrous material such as sulfite pulp, after 75 which the mixture is fabricated into sheets, as desired. The rubber or celluloid is dissolved in an appropriate solvent, such as benzol or acetone, to provide a fluid plastic solution with which the fibrous material may 80 be mixed. The mixture may be felted, pressed or otherwise formed into sheets of the desired thickness and the solvent then evaporated, which leaves the sheets rigid and pervious to a predetermined degree, with the 85 fibers bonded together. The amount of bonding material employed depends upon the nature of the fibrous material used and upon the rigidity required. When cotton linters are used, sufficient plastic composition 90 may be used to coat the fibers to protect them from attack by the electrolyte, whereas in the treatment of sulfite pulp a smaller amount of the composition will usually suffice to bond the fibers and provide the required rigidity for a separator.

Bituminous material rendered fluid by heating, such as asphalt, may also be employed as a bonding and reinforcing agent to be incorporated with the fibrous material 100 before or after the formation of the sheet. A jelly-forming substance, such as sodium silicate, may also be employed by itself as a bonding and reinforcing agent in the manner described, or may be combined with the 105 rubber, celluloid or bitumen. The sodium

silicate in the separator when acted upon by the electrolyte of the battery becomes gelatinous silicic acid, bonding, the loosely felted fibers together and filling the pores between them. This bonding agent thus prevents creepage of active material and growths through the separator but, being permeable to electrolytic action, permits free diffusion of the electrolyte and passage of electric current through the separator. The 10 felted body of fibers has tortuous through passages or pores uniformly distributed throughout its area, and the rubber, celluloid and similar bonding material is so incorporated as not to obstruct these pores. The 15 cementitious material employed constitutes the sole means, aside from the felted arrangement of the lengthy fibers, for bonding these fibers together, since the treated fibrous 20 material used is initially free from the natural gums, resins, etc.

On the other hand, sheets may first be formed from appropriate acid-resistant fibrous material and then impregnated with 25 an acid-resistant plastic bonding agent, such as rubber or celluloid dissolved in an appropriate solvent. The solvent is then evaporated, which sets the bonding material and leaves the sheet porous to the desired 30 degree. The sheet may also be treated with sodium silicate, as already described.

The rubber bonding material may be vulcanized in the separators by treating such 35 rubber-bonded separators with a solution of sulfur monochlorid in an appropriate solvent such as carbon bisulfide, drying the separators, washing them first in sodium bicarbonate solution and then with water, and finally drying them. The sheets of 40 fibrous material may be treated initially with rubber and sulfur or other suitable vulcanizing agent in an appropriate solvent, such as carbon bisulfide. After evaporating the solvent, the separator is heated to about 45 140° C. for from 2 to 5 hours to vulcanize the rubber.

The improved separators, made from bonded chemically treated but uncalendered fibrous materials such as sulfite pulp and 50 cotton linters, possess the advantages of the best wooden and other separators in lightness, thinness and about the same low resistance to current in the battery. But they are much superior to such separators because they are less expensive, are more uniform in porosity and freedom from detrimental substances and fillers such as those used in papers, and having no grain, are of the same strength in all directions. To 55 effectively reduce splitting and warping, wooden separators must be kept moistened, whereas the characteristics of the improved separator herein disclosed do not change even when kept in dry condition indefinitely. These separators may therefore be assem-

bled in dry condition in batteries and shipped at less expense and inconvenience, and stored without danger of deterioration.

I claim:

1. A storage battery separator consisting 70 of a uniformly pervious sheet formed of fibers uniformly free from substances which detrimentally affect the operation of a battery, such sheet having cementitious material incorporated therein bonding said fibers 75 together.

2. A storage battery separator comprising fibers felted into a sheet and bonded together solely by acid-resistant material, such sheet being rigid, of uniform strength in 80 all directions, uniformly pervious to electrolyte, and uniformly free from substances that detrimentally affect the operation of a battery.

3. A storage battery separator consisting 85 of a sheet formed of sulfite pulp fibers bonded together and uniformly free from substances detrimental in the operation of a battery.

4. A storage battery separator consisting 90 of a rigid uniformly pervious sheet formed of felted sulfite pulp fibers bonded together by acid-resistant material and uniformly free from substances detrimentally affecting the operation of a battery. 95

5. A storage battery separator according to claim 2, in which such bonding material is vulcanized but does not obstruct the pores of said sheet.

6. A storage battery separator according 100 to claim 2, in which the pores of such sheet contain a jelly-forming substance permeable to electrolytic action.

7. A storage battery separator consisting 105 of rigid porous sheet comprising cotton linters bonded together by acid-resistant material.

8. A method of making storage battery separators that comprises incorporating an acid-resistant bonding agent in a body of 110 fibers free from substances detrimental in the operation of a battery, and forming such material into sheets adapted for use as separators.

9. A method of making storage battery 115 separators that comprises the step of incorporating bonding material in a body of fibers that have been subjected to treatment uniformly freeing them of substances detrimentally affecting the operation of a battery. 120

10. A method of making storage battery separators that comprises mixing acid-resistant plastic material with a body of fibers freed from substances detrimental in the 125 operation of a battery, and forming such mixture into sheets.

11. A method of making storage battery separators that comprises incorporating fluid bonding composition in a body of fibers

freed from substances detrimental in the operation of a battery, and solidifying such bonding composition.

12. A method of making storage battery separators that comprises incorporating fluid bonding composition containing a volatile solvent in a body of fibers uniformly free from substances detrimental in the operation of a battery, and evaporating such solvent.

13. A method of making storage battery separators that comprises incorporating acid-resistant bonding material in a body of sulfite pulp fibers, and forming the same into separator sheets.

14. A method of making storage battery separators that comprises incorporating vulcanizable bonding material in a body of fibers, forming the same into sheets, and vulcanizing such bonding material.

15. A method of making storage battery separators that comprises incorporating bonding material and jelly-forming material in a body of fibers uniformly freed from substances that detrimentally affect the operation of a battery.

In testimony whereof, I affix my signature.

RAYMOND C. BENNER.